

Feb. 28, 1928.

1,660,960

G. R. GREENSLADE

FLEXIBLE STAY BOLT AND METHOD OF MAKING

Filed Feb. 18, 1927

*Fig. 1.*



*Fig. 2.*



INVENTOR

Grover R. Greenslade  
by his attorneys  
Bynes, Stettinius, Parmelee

## UNITED STATES PATENT OFFICE.

GROVER R. GREENSLADE, OF PITTSBURGH, PENNSYLVANIA, ASSIGNOR TO FLANNERY BOLT COMPANY, OF PITTSBURGH, PENNSYLVANIA, A CORPORATION OF DELAWARE.

## FLEXIBLE STAY BOLT AND METHOD OF MAKING.

Application filed February 18, 1927. Serial No. 169,256.

This application is a continuation in part of my copending application, Serial No. 118,515, filed June 25, 1926.

The present invention relates to flexible staybolts and method of making, and more especially to a staybolt having a hardened head, and also to the combination of a headed staybolt and a seat therefor, one of which has an anti-friction bearing surface.

10 Flexible staybolts are employed in steam boilers, and more especially in locomotive boilers, in order to allow relative movement between the wrapper sheet and fire sheet. Referring particularly to a locomotive boiler, 15 the fire box is formed within the boiler, the side walls and top of the fire box being bounded by the water space of the boiler. The sheet between the fire space and the water space of the boiler is usually called 20 the fire sheet. The sheet around the outside of the boiler is usually called the wrapper sheet. These two sheets are tied together by staybolts. Due to unequal expansion of the parts under variations in temperature there 25 may be a considerable movement between the wrapper sheet and fire sheet, amounting, at times, to perhaps one-quarter of an inch. This movement takes place principally in the planes of the fire and wrapper sheets. 30 In order to permit such movement without damage to the staybolts, the "flexible" staybolts have been employed. The usual so-called flexible staybolt consists of a bolt which is threaded into the fire sheet at one 35 end. The other end of the bolt has an enlarged head which is seated in a sleeve secured to the wrapper sheet, the head of the bolt being covered by a cap screwed or otherwise secured to the sleeve. This permits a 40 ball-and-socket motion between the bolt head and its seat in the sleeve. The fire sheet is usually of thinner material than the wrapper sheet. It is also maintained at a higher 45 temperature in service. Moreover, it would not be practicable to have caps projecting into the fire box from the fire sheet. For this reason the wrapper sheet end only of the staybolt has been provided with the ball-and-socket joint, it being found that the 50 thinner fire sheet has sufficient flexibility to allow the deflection of the staybolt.

When locomotives were first constructed the boilers were small and operated at rela-

tively low pressures, and practically all of the staybolts were "rigid" staybolts, that is, 55 staybolts which were screwed or otherwise rigidly secured to both the wrapper and fire sheets. It was found, however, that as the size of the boilers and the steam pressure were increased, serious breakage took place 60 with the rigid staybolts. This breakage occurred usually at the ends of the bolts where they were screwed into the wrapper and fire sheets, and most commonly at the wrapper sheet end of the bolt. Some breakage, however, took place at the fire sheet end. In order to meet this condition, the flexible type of staybolt was developed, such staybolts usually being of the type shown in the Tate Patent No. 813,120 of February 20, 1906. 70 It was found that the use of the ball-and-socket connection at the wrapper sheet not only prevented the breakage of the bolts at the wrapper sheet end, but also diminished the breakage of the bolts at the fire sheet end. 75 as well. The reason for this can be seen by an analysis of the conditions surrounding the use of the rigid staybolt. The rigid staybolt is rigidly screwed into both the wrapper and the fire sheet. Therefore, upon 80 relative movement of the two sheets the staybolt is subjected to the stresses of a beam rigidly secured at both ends and the rigid staybolt is bent with a reverse curve. In the flexible type of staybolt, however, one end is 85 free, so that upon relative movement of the two sheets the staybolt behaves as a beam rigidly secured at one end only, the other or loaded end being rotatably free. Therefore, for the same relative movement between the wrapper and fire sheets, the 90 amount of bending moment to which the flexible staybolt is subjected is only about half of that to which the rigid staybolt is subjected.

95 The flexible staybolts such as shown in the Tate patent solved the staybolt problem for the time being. However, in recent years the size of the locomotive boilers and the steam pressures have been greatly increased 100 so that the staybolts have not only been subjected to greater relative lateral movements of the fire and wrapper sheets, but also the tension on the bolts has been greatly increased. The staybolt breakage again began 105 to be serious. It was found that the Tate

flexible staybolts which were practically unbreakable in locomotive boilers in vogue when the Tate bolts were first introduced, were subject to breakage in the more modern 5 large locomotives.

I have found that the breakage appears to have been due to two factors, namely, the increased tension on the bolts and the increased relative movement between the fire 10 and wrapper sheets. The tension on the staybolts at certain parts of the boilers has been increased to a point where the staybolt head has been drawn against its sleeve so tightly as to reduce and even prevent the 15 ball-and-socket slippage between the head and its seat in the sleeve. This increase in tension has practically defeated the object of the flexible staybolt, because a bolt which has its head frictionally locked against its 20 seat acts as a rigid bolt, and the shank of the bolt is subjected to the same amounts of stress as a rigid bolt. This has resulted in breakage of the flexible staybolts, particularly at the neck just below the head of 25 the bolt, and also near the fire sheet end of the bolt, these two points being the points of maximum bending to which the rigidly locked bolts have been subjected.

I have found that this breakage may be 30 prevented by making one or both of the contacting surfaces between the bolt member and the sleeve member of the assemblage of a very hard metal. If one or both members are made of a hard metal, I have found that 35 the locking which took place between the relatively soft metal surfaces of the bolt head and sleeve may be prevented for boiler pressures now encountered. This condition is preferably secured by locally hardening 40 the head of the bolt where it contacts with the sleeve. This condition could not be remedied by using a bolt wholly of a hard material, as will be apparent from the following considerations. In practice in the 45 United States, staybolts have been practically universally made of wrought iron because of its ductility and resistance to corrosion. Some roads, particularly the Canadian railroads, have used a very low carbon mild 50 ductile steel for staybolts. These materials are necessary because a considerable amount of ductility is required in the staybolt. The yield point of the material should not be too high. The staybolt, particularly at the fire 55 sheet end, is subjected to deformation which may exceed the elastic limit of the material, and therefore to minimize or prevent breakage from fatigue a mild ductile metal should be used. Also, it is practically impossible in 60 applying the staybolts to the cold boiler to screw them in so that when the boiler is heated up and the tension is applied to the bolts, that the tension is uniformly distributed over all of the staybolts. Some of 65 the staybolts will inevitably be put under

greater tension and the staybolt metal should be ductile so as to allow the staybolts to yield and adjust themselves to the boiler.

While it is preferred to surface harden the bolt head, the sleeves may be surface 70 hardened. The sleeves, however, should still be made of a material which permits the body of the sleeve to be malleable and ductile. In removing the caps for inspection purposes or replacement of bolts, it is found 75 that the caps often stick tightly and the workmen strike the caps with hammers to loosen them, thus subjecting the sleeves to severe treatment, so that the sleeves should be made of material which will not readily 80 fracture. For this reason it is preferred to have the body of the bolt and the body of the sleeve of the milder metals now used, and to surface harden the bearing surfaces between the bolt head and sleeve. 85

Another weakness in flexible staybolts as usually heretofore made has been brought out by the increased demands on staybolts by modern locomotive practice. This weakness has been the tendency of the bolts to 90 crack just under the heads. In making the flexible staybolts, according to the usual practice, a round bar of staybolt iron (or steel) of the proper length has several inches 95 of one end heated. The bar is then clamped in a machine, leaving projecting sufficient metal to form the head. A die is then brought against the heated end and gathers or mashes the metal into a generally spherically shaped ball or bunch on the end of the bar. The roughly formed upset head is then 100 finished by a forging operation usually carried out by placing the head in hammer dies which strike forming blows on the head to shape it to spherical form. The head, however, may be entirely forged by forming dies. The dies of the hammer or forging machine are cold and the metal has been 105 cooling from the time the head was first upset, so that the finish of the forming operation is often carried out on metal, particularly at the surface, which may have dropped in temperature below the best forging temperature. Since the forging is a 110 hand operation, it is practically impossible to see that the workmen always carry out the forging at the best forging temperature. The result has been that the metal, particularly at the surface of the head and of the 115 neck where the head joins the shank of the bolt, has in many cases had its grain structure seriously impaired. Photo-micrographs have shown that while the iron at the interior of the head has the normal grain structure with bands of slag running longitudinally of the bolt, at the forged surfaces the grains seem to be distorted and broken up. The slag bands are also somewhat 120 broken up. The result has been that the surface metal has been weakened so that cracks 125

130

could start in it and penetrate into the metal at the interior of the bolt. As is well known, a crack tends to continue from weakened metal into normal metal.

6 I can overcome this weakness by restoring the grain structure without surface hardening the metal of the bolt head, although I prefer to combine the surface hardening and grain restoration in the same operation.

10 The preferred process of making stay-bolts in accordance with my invention will now be described, reference being had to the accompanying drawings, in which—

15 Figure 1 is an elevation partly in section showing a staybolt assemblage applied to the boiler; and

Figure 2 is a detailed sectional view of a sleeve showing a modification.

20 Referring to the drawings, the wrapper sheet 1 and fire sheet 2 are shown as being connected by a flexible stay-bolt assemblage which comprises the usual bolt member 3, sleeve 4 and cap 5. The bolt 3 is threaded at 6 into the fire sheet 2, the end 7 being 25 riveted over in the usual manner. The sleeve 4 is threaded at 8 into the wrapper sheet 1. The bolt 3 has the usual enlarged spherical head 9 which engages the seat 10 of the sleeve 4.

30 The parts as above described are those of the well known Tate bolt employing a threaded sleeve. The invention, however, is not limited to the Tate bolt but may be embodied in various other types of flexible stay-bolts, such, for example, as the so-called 35 "button head" or the "taper head" type of flexible crownstay in which a spherically surfaced nut is screwed on the wrapper sheet end of the bolt to make contact with the sleeve, or may be embodied in the so-called 40 "welded type" of staybolt assemblages in which the sleeves, instead of being threaded to the wrapper sheet, are welded to the wrapper sheet.

45 While the bearing seat for the staybolt head is usually provided in a sleeve attached to the boiler sheet as shown for example in the Tate Patent No. 813,120, of February 20, 1906, the bearing seat may be otherwise 50 formed, for example, as shown in the Menne Reissue No. 14,796, of January 27, 1920, in which the bearing seat is formed directly in the outer boiler sheet.

In my improved staybolt assemblage, one 55 or both of the contacting surfaces of the bolt member 3 and sleeve or seat member 4 are hardened so as to prevent the frictional sticking under heavy tensions on the bolt. The motion of the parts is not sufficient so 60 that the surface hardening is necessary to resist wear. The surface hardening is done for the purpose of preventing the parts from binding, which I have found to take place with metal surfaces having the ductility and 65 mildness demanded for the body of the stay-

bolt. As indicated in the drawings, the head of the staybolt has its surface carburized, as indicated by the shading 11. This surface carburization is usually applied over the entire head of the bolt and a short distance 70 along the neck 12. The sleeve 4 is shown as having its surface hardened by carburization, as indicated at 13.

75 While both the head and sleeve are shown as having their contact bearing surfaces carburized, one only need be carburized, preferably the bolt head.

In Figure 2 is illustrated a modification in which the sleeve body, instead of having a hardened seat formed by surface carburizing, has a hardened seat formed by an inset 14 of hard steel or of other suitable hard metal or alloy.

80 The preferred process of making the stay-bolts is as follows:

85 A bar of staybolt iron of the proper length has its end heated for several inches to a forging heat and the end is then upset to form a roughly spherical head. This upsetting operation, if properly carried out, should not destroy what is commonly called the fibrous constitution of the iron. Staybolt iron is made from wrought iron containing a certain amount of slag. It is 90 found that the presence of the slag gives the iron greater resistance to corrosion and also a more fibrous nature than that of the so-called "dry" wrought iron from which the slag is practically eliminated. In making the staybolt iron bars, a number of muck 95 bars are either box piled or slab piled and then re-rolled so as to give the staybolt iron the so-called fibrous structure in which the layers of slag lie as bands longitudinally of the bar, separating what are known as 100 fibers of the iron. The iron fibers are, of course, microscopically made up of a series of grains partially sheathed by bands of slag. The iron is stronger lengthwise of the 105 so-called fibers. If the upsetting operation 110 is properly carried out, the fibrous condition of the iron will persist in the head, the so-called fibers in the head being bulged out somewhat like the layers of an onion but still preserving the general longitudinal direction.

115 After the metal is upset to form the rough head, the head is forged to finished spherical form in the usual way by finishing dies.

120 The staybolts are then treated to restore the grain structure and to surface harden the heads. This is preferably done by immersing the heads of the staybolts in a molten bath of potassium cyanide at a temperature of about 800° C. for about ten minutes. This brings the heads quickly to a bright red heat which serves to normalize the metal, that is to say, it restores to a normal condition the grain structure which may have been 125 damaged by the forging operation. The 130

cyanide treatment also serves to carburize the surface of the staybolt head but without carburizing the interior of the head or the metal in the shank.

5 During this carburizing operation only the heads of the bolts are dipped into the molten cyanide bath. As soon as the bolts are removed from the cyanide bath they are immediately quenched in water. This serves to 10 increase the yield point and ultimate tensile strength of the metal throughout the head, particularly at the neck, at which place failure frequently takes place. Since the hardened surface prevents the head of the stay- 15 bolt from binding in the sleeve, the metal in the head and neck is not subjected to distortion due to bending moments, and hence can be made harder and stiffer than the metal in the shank and at the fire sheet end of 20 the bolt body, where the metal is subjected to bending. This treatment, therefore, results in localizing the hardness and the increased yield point and ultimate tensile strength where they are most desired, leaving 25 the original ductility of the metal localized in the shank and fire sheet end.

While for practical shop operation the heating of the metal in the cyanide bath is usually sufficient to restore any damaged 30 grain structure, the process may be modified, if desired, by heating the staybolt heads to a somewhat higher temperature, say, about 900° centigrade, and thereafter either immediately immersing them in the molten cyanide bath or quenching and then immersing them in the molten cyanide bath. Such preliminary treatment to a higher temperature can more completely restore a badly damaged grain structure.

40 I have found that with staybolt iron there is practically no objectionable grain growth encountered in heating the heads of the bolts in accordance with the ordinary shop practice of my method as above described 45 and without any extraordinary precaution. Staybolt iron in this respect differs somewhat from steels, and particularly the higher carbon steels.

For general purposes it is usually sufficient 50 to harden the bolt heads only. However, if desired, the seating surface of the sleeves may be hardened, in which case the hardening of the bolt heads may be omitted or both the bolt heads and sleeves may be hardened. 55 The sleeves are preferably hardened by a local cyanide carburizing treatment, leaving the body of the sleeve of the usual mild, tough sleeve steel stock. However, the hardened surface of the sleeve may be provided 60 in other ways, as, for example, by the inset 14 shown in Figure 2, or the entire sleeve may be made of a hardened alloy steel, as contrasted with the practice heretofore of using a mild steel for the sleeves. Such 65 hard alloy steels will give an excellent bear-

ing surface and resist hammering without fracture, but they are, however, relatively expensive.

While a cyanide carburizing treatment is preferred for hardening the contact surfaces, 70 other hardening treatments might be employed, such, for example, as carburizing by other processes such as the pack process, or by plating, such as with chromium, or chromium alloys, or other plating metals. 75

The bearing surface of the bolt head or the bearing surface of the sleeve should be much harder than the metal of the main body of the bolt proper. By the expression "much harder", I mean a degree of hardness comparable to that obtained by carburizing and quenching, by the use of hard steels, or by chromium plating or the like, as distinguished from such differences in hardness as may have existed between the usual unhardened or mild steel sleeves and the wrought iron staybolts as heretofore made. 85

I am aware of the suggestion of the use of copper liners or washers between staybolt heads and sleeves to prevent corrosion 90 and reduce friction. I have found, however, that with the enormous tensiles to which the staybolts are subjected in modern locomotive boilers, such copper liners are 95 worse than useless, as they simply serve to lock the staybolt head against rotational movement in the sleeve. The softer metals under the greater pressures seem to have their surfaces forced into such intimate or microscopically interlocking contact that 100 while the staybolt head might turn for lighter pressures it is rigidly locked at heavy pressures. I have found, however, that when one or both of the contacting surfaces are hardened, this interlocking is prevented, at 105 least to such an extent that the heads are free to turn in the sleeves with the staybolt tensiles even greater than those encountered in modern locomotive practice. This has been demonstrated by tests in which the 110 ordinary staybolts have been compared with my improved staybolts. In such tests a heavy tension, equal or exceeding that to which the staybolts are subjected in modern locomotive practice, is applied to a staybolt. 115

The headed end of the staybolt is held in a sleeve which is rigidly mounted. The lower end of the staybolt to which tension is applied is given a continued slight oscillatory movement at right angles to the axis of the bolt. It has been found that while the ordinary staybolts may stand, say, from 150,000 to 250,000 oscillations before breaking, my staybolts under exactly the same tensions and amplitude of oscillations, will 120 stand from 2,000,000 to 5,000,000 oscillations before breaking. 125

I believe that the increased performance of my staybolts is jointly contributed to by the minimizing of friction or the preventing 130

of locking under heavy pressure effected by the hardened contact surfaces, by the restoring of any damaged grain structure, particularly at the point where the head joins the neck, and by the increased strength given to the neck and head by quenching.

While all three of these factors are apparently necessary for the best results, it is obvious that not all of them need be present. For example, the performance of the staybolts may be greatly improved by restoring the damaged grain structure without quenching and without surface hardening, or the surface may be hardened without quenching, as, for example, by electroplating, or the heads and necks may have their hardness and strength increased by quenching without carburizing or plating.

While I have described the problems encountered and the preferred embodiments of my invention, at considerable length, it is to be understood that the invention is not limited to its preferred embodiments but may be otherwise embodied within the scope 25 of the following claims.

I claim:

1. The combination of a headed staybolt and a seat therefor having cooperating bearing surfaces, at least one of which is much harder than the metal of the main body of the bolt member.

2. The combination of a headed staybolt and a seat therefor having cooperating bearing surfaces, at least one of which is formed 35 by a carburized hardened surface.

3. The combination of a headed staybolt and a seat therefor having cooperating bearing surfaces, the bearing surface of the bolt head being much harder than the metal of the main body of the bolt.

4. The combination of a headed staybolt and a seat therefor having cooperating bearing surfaces, the bearing surface of the bolt head being carburized to a surface hardness 45 much harder than that of the metal of the body of the bolt.

5. A staybolt assemblage comprising a headed bolt member and a sleeve member having cooperating bearing surfaces, and a 50 cap secured to the sleeve member and covering the bolt head, at least one of the cooper-

ating bearing surfaces of the bolt and sleeve member being much harder than the metal of the main body of the bolt member.

6. A staybolt having an enlarged forged 55 head, the bolt head being normalized, surface carburized and quenched, whereby there is imparted to the head a normal grain structure having a greater strength than that of the shank of the bolt and hardened bearing surface.

7. A staybolt having an enlarged head and a neck of much greater surface hardness and strength than the shank of the bolt.

8. The process of making staybolts which 65 comprises upsetting and forging an enlarged head on the bolt body, heating the bolt head in contact with a carburizing agent for a sufficient time to restore grain structure damaged by the forging operation and to 70 carburize the surface of the bolt head which contacts with the sleeve, and thereafter quenching, leaving the metal of the bolt shank substantially unaffected.

9. The process of making a staybolt which 75 comprises upsetting and forging an enlarged head on the bolt body, immersing the head in a heated cyanide bath for a sufficient time to carburize the surface and restore damaged grain structure, and thereafter quenching to 80 harden the carburized surfaces and locally increase the strength of the body of the head and neck, leaving the metal of the bolt shank substantially unaffected.

10. The process of making staybolts which 85 comprises upsetting and forging an enlarged head on the bolt body, carburizing the surface of the bolt head which contacts with the sleeve in the staybolt assemblage, and quenching, whereby such surface is rendered 90 much harder than the metal of the main body of the bolt.

11. A staybolt having an enlarged head which is forged, normalized and surface hardened.

12. A staybolt having an enlarged head provided with a bearing surface much harder than the metal of the main body of the bolt.

In testimony whereof I have hereunto set 100 my hand.

GROVER R. GREENSLADE.